

1

2,861,063

## ODOR STABILIZATION OF SULFUR-CONTAINING ORGANIC MATERIALS

Fredrick L. Jonach, Kew Gardens, N. Y., assignor to Esso Research and Engineering Company, a corporation of Delaware

No Drawing. Application September 22, 1955  
Serial No. 536,013

5 Claims. (Cl. 260—139)

This invention relates to the odor stabilization of sulfur-containing organic materials which normally evolve hydrogen sulfide and more particularly relates to a method for stabilizing such materials by treating them with lead peroxide ( $PbO_2$ ), to the resultant stabilized products and to lubricants containing the stabilized products as additives.

Many organic sulfur-containing compounds normally evolve hydrogen sulfide during storage, transportation, or use. Because of the obnoxious odor of hydrogen sulfide, this evolution is quite objectionable. Frequently, it is desired to use such compounds as additives for mineral oil compositions, such as lubricating oils, to impart to the composition various desired properties, such as extreme pressure properties, anti-corrosive properties, detergent properties, and the like. However, compositions containing even small amounts of unstable sulfur-containing compounds will evolve hydrogen sulfide. Users of such compositions object to these odors and consequently the saleability of the product is impaired. Many organic compounds that have been sulfurized or phosphosulfurized by treatment with sulfur, sulfides of phosphorus and the like show this characteristic instability with respect to hydrogen sulfide evolution.

Numerous attempts have been made in the prior art to stabilize such sulfur-containing compounds or compositions including these compounds. None of these prior art methods have been entirely effective and they have been especially ineffective with phosphosulfurized hydrocarbons which in general are extremely potent  $H_2S$  evolvers. It is unfortunate that heretofore it has not been possible to effectively stabilize these phosphosulfurized hydrocarbons since not only are they inexpensive but they are also among the most potent detergent and oxidation inhibitor additives known for lubricating oil compositions.

It has now been found that the evolution of hydrogen sulfide from unstable sulfur-containing organic materials may be effectively eliminated or at least partially reduced by treating these materials with lead peroxide ( $PbO_2$ ). The lead peroxide treatment also reduces the corrosivity of the sulfur-containing organic materials.

## THE SULFUR-CONTAINING ORGANIC MATERIALS

The present invention is especially directed to those sulfur-containing organic compounds which normally evolve hydrogen sulfide and which are useful as lubricating oil additives and are oil-soluble, although it will be understood that the method of this invention is applicable to other sulfur-containing organic compounds which normally evolve hydrogen sulfide.

One particular class of sulfur-containing organic compounds which are useful as lubricating oil additives are the sulfurized and/or phosphosulfurized hydrocarbons. These hydrocarbon materials may be paraffins, such as bright stock residuums, lubricating oil distillates, petrolyums, paraffin waxes, etc.; olefins, such as isobutylene,

2

acrolein, decene, dodecene, cetene, octadecene, etc.; olefin polymers having molecular weight ranges from about 100 to 50,000, particularly from about 500 to 10,000, such as those of ethylene, propylene, butylene, isobutylene, amylanes, etc.; diolefins, such as butadiene, isoprene, chloroprene, cyclopentadiene, terpenes, etc.; acetylenes; copolymers of low molecular weight monoolefins and diolefins having molecular weight ranges of about 1,000 to 30,000; aromatics, such as benzene, naphthalene, anthracene, toluene, xylene, diphenyl, etc.; alkyl aromatics; cyclic aliphatics; petroleum fractions; condensation products of halogenated aliphatic hydrocarbons with an aromatic compound and the like.

Another class of sulfur-containing organic compounds which are useful as lubricating oil additives are sulfurized and/or phosphosulfurized oxygen-containing organic compounds. Included in this group are sulfurized and/or phosphosulfurized animal and vegetable oils, fats, rosins, resin and the acid ester hydrogenated and lower alkyl derivatatives thereof. Included in this class are products such as sulfurized sperm oil, phosphorus sulfide treated rosin, rosin derivatives such as methyl abietate and the like, for example, the products sold under the trade name "Abalyn," "Hercolyn" and the like, as well as various sulfur and/or phosphorus sulfide treated organic acids, methyl esters, etc., derived from these products and from lanolin, degras, tall oil, and the like. Such materials as have been described above are well known to those skilled in the art.

30 The sulfurization and/or phosphosulfurization of hydrocarbons, oxygen-containing organic compounds and the like are also well known in the art. Sulfurization is generally accomplished by reacting the organic compound with elemental sulfur. The sulfides of phosphorus which can be employed for phosphosulfurization include  $P_2S_3$ ,  $P_2S_5$ ,  $P_4S_3$ ,  $P_4S_5$ , or other phosphorus sulfide and is preferably phosphorus pentasulfide ( $P_2S_5$ ). Mixtures of two or more phosphorus sulfides may also be employed as well as mixtures of elemental phosphorus sulfur.

40 The sulfurization and/or phosphosulfurization reaction is conveniently carried out at an elevated temperature of about 200 to 600° F., preferably about 300 to about 550° F., using in general about 2 to about 5 molecular proportions of the organic compound to 1 molecular proportion of sulfur or phosphorus sulfide in the reaction. The reaction will generally be carried out until the maximum amount of sulfur or phosphorus sulfide has been added to the organic compound although this is not essential. The reaction time is not critical and the time required to cause the maximum amount of sulfur or phosphorus sulfide to react will vary with the temperature. A reaction time of 2 to 10 hours is frequently necessary and, if desired, the reaction product may be further treated by blowing with steam, alcohol, ammonia, or an amine at an elevated temperature of about 200° F. to improve the odor thereof to a certain extent. The sulfur-containing organic materials of this invention will generally contain at least 1.0% and usually at least 2.0% by weight of chemically combined sulfur.  $P_2S_5$  treated polyisobutylenes having molecular weights in the range of about 500 to 25,000, particularly about 500 to 2,000, are especially stabilized effectively in accordance with this invention by treatment with  $PbO_2$ .

THE TREATMENT WITH  $PbO_2$ 

70 The odor stabilization of the sulfur-containing organic materials in accordance with this invention is accomplished by treating these materials with lead peroxide ( $PbO_2$ ). In general, the unstable sulfur-containing organic materials will be treated with a small amount of  $PbO_2$  at an elevated temperature for an extended period of time. In the stabilization reaction, the reaction

variables, namely, temperature, time and proportion of  $PbO_2$ , are interchangeable to a certain extent. Generally more effective stabilization will be obtained when using higher temperatures, longer reaction times and greater proportions of  $PbO_2$ .

Elevated temperatures in the range of about 80° to 400° F. are generally effective in the stabilization reaction carried out in accordance with the present invention. Temperatures in the range of about 150° to 350° F. are preferred and a temperature of about 300° F. has been shown to be exceedingly effective. As to the reaction time, generally a period of at least about one hour is required. Effective stabilization is obtained when utilizing reaction times of about 8 to 24 hours, preferably about 12 to 16 hours. In general, about 0.5 to 50% by weight of  $PbO_2$  will be employed, based on the sulfur-containing organic material to be stabilized. Proportions of  $PbO_2$  in the range of about 5% to 30% by weight, based on the sulfur-containing organic material, are preferred and exceedingly effective results are obtained when utilizing about 10 to 25% by weight of  $PbO_2$ .

If the sulfur-containing organic material is liquid under the treating conditions, the treating reaction may be carried out without a solvent. However, in general, it is preferred to carry out the stabilization reaction of the present invention in the presence of a solvent for the sulfur-containing organic material. Hydrocarbon solvents are preferred, with a mineral lubricating oil being the preferred solvent since normally the sulfur-containing organic materials useful as lubricating oil additives are marketed as additive concentrates consisting of the additive in a diluent mineral oil. The stabilization reaction is preferably carried out with intimate mixing of the reactants, such as by stirring the reaction mixture. It is preferred to utilize  $PbO_2$  in a finely divided form (such as a powder) to provide ready contact between it and the sulfur-containing organic materials. After the stabilization reaction, any unreacted  $PbO_2$  may be filtered from the reaction mixture. The stabilized reaction products of this invention will in general contain in the range of about 0.1 to 10 wt. % of lead as a result of the stabilization reaction.

The invention will be more fully understood by reference to the following examples. It is pointed out, however, that the examples are given for the purpose of illustration only and are not to be construed as limiting the scope of the present invention in any way.

#### Example I

*The sulfur-containing organic material to be stabilized in accordance with the present invention.*—A polyisobutylene of about 1100 Staudinger molecular weight was reacted with about 10% by weight of  $P_2S_5$  (based on the polyisobutylene) at a temperature of about 425° F. for about 8 hours. The phosphosulfurized polyisobutylene was diluted with a mineral lubricating oil to form two additive concentrates, product A containing about 40% and product A' containing about 50% by weight of the phosphosulfurized polyisobutylene.

*Treatment of Product A with  $PbO_2$ .*—100 grams of product A were then stirred with 10 grams of powdered  $PbO_2$  at a temperature of about 190° F. for about 30 hours. The resultant stabilized reaction product, hereinafter referred to as product B, was blended with a solvent refined mineral lubricating oil (having an S. U. S. viscosity at 210° F. of about 45 seconds and hereinafter referred to as the base stock) to form a lubricating oil composition containing about 10 vol. percent of product B. This composition was diluted with normal heptane and filtered through "Celite" filter aid. The heptane was removed, giving a light-colored lubricating oil composition of excellent odor characteristics.

A second lubricating oil composition was prepared

using product A. This second composition consisted of about 10 vol. percent of product A in the base stock. These two compositions had the following properties:

TABLE I

|                                | 10 vol. percent of product A in base stock | 10 vol. percent of product B in base stock |
|--------------------------------|--------------------------------------------|--------------------------------------------|
| Odor rating                    | Bad                                        | Good                                       |
| Sulfur (weight percent)        | 0.59                                       | 0.50                                       |
| Phosphorus (weight percent)    | 0.16                                       | 0.15                                       |
| Lead (weight percent)          |                                            | 0.29                                       |
| 15 Neut. number                | 1.4                                        | 2.1                                        |
| Sap. number                    | 4.3                                        | 3.4                                        |
| Lead acetate test <sup>1</sup> | 10+                                        | 0                                          |
| Color (tag-Robinson)           | 7½                                         | 7½                                         |
| Vis./100° F. (S. U. S.)        | 282.4                                      | 294.9                                      |
| Vis./210° F. (S. U. S.)        | 53.6                                       | 55.1                                       |

<sup>1</sup> The lead acetate test is an effective test for determining the stability as to  $H_2S$  evolution of compositions containing sulfur-containing organic materials. This test is carried out as follows: 800 cc. of the oil composition are placed in a 1-quart bottle and heated at 120° F. for one hour. Then a piece of paper moistened with saturated lead acetate solution is exposed to the blend for a period of 5 minutes. The resultant lead sulfide stain is rated for its intensity, a rating of 10 being a dark stain with a trace of silvery overlay, a rating of 0 being no stain, and a rating of 10+ being a stain with considerable silvery overlay.

It will be noted that the method of the present invention is exceedingly effective in stabilizing a sulfur-containing organic material such as phosphosulfurized polyisobutylene. More specifically, it will be noted that the oil composition containing product B of the present invention had a 0 rating in the lead acetate test whereas the oil composition containing product A had a rating of 10+ in the lead acetate test.

#### Example II

Product A' was stabilized, in accordance with the present invention, utilizing varying proportions of powdered  $PbO_2$  and varying reaction times to produce stabilized additives as shown below.

TABLE II

| 50                  | Stabilization reaction conditions |                          |                                        |                       |                      | Lead acetate test rating <sup>1</sup> |
|---------------------|-----------------------------------|--------------------------|----------------------------------------|-----------------------|----------------------|---------------------------------------|
|                     | Weight of product A' (gms.)       | Weight of $PbO_2$ (gms.) | Percent of $PbO_2$ based on product A' | Reaction temp. (° F.) | Reaction time (hrs.) |                                       |
| Sample of product A | 0                                 | 0                        | 0                                      |                       |                      | 10                                    |
| 181                 | 38                                | 20.0                     | 300                                    | 8                     |                      | 7                                     |
| 55 161              | 32                                | 20.0                     | 300                                    | 24                    |                      | 0                                     |
| 362                 | 72                                | 20.0                     | 300                                    | 12                    |                      | 0                                     |
| 362                 | 72                                | 20.0                     | 300                                    | 16                    |                      | 0                                     |

<sup>1</sup> The lead acetate test was carried out in this example in the following manner: The treated product was blended with the base oil to form a composition of 10 weight percent of the treated product and 90 weight percent of the base oil. The resultant composition was then rated for  $H_2S$  evolution as described in Example I.

It will be noted that the evolution of hydrogen sulfide from product A' was reduced by treating it with  $PbO_2$  in accordance with the present invention. When reaction times of 12 hours or greater were employed, there was no detectable evolution of  $H_2S$  from the treated product in the lead acetate test.

#### Example III

In this example, product A was blended with the base stock to prepare compositions containing about 10 wt. percent of product A in the base stock. Portions of this composition were treated with powdered  $PbO_2$  at several

different reaction temperatures to prepare stabilized compositions as shown below.

TABLE III

| Stabilization reaction conditions <sup>1</sup> |                                   |                                                |                      |                    | Lead acetate test rating <sup>2</sup> |
|------------------------------------------------|-----------------------------------|------------------------------------------------|----------------------|--------------------|---------------------------------------|
| Weight of product A (gms.)                     | Weight of PbO <sub>2</sub> (gms.) | Percent of PbO <sub>2</sub> based on product A | Reaction temp. (°F.) | Reaction time (F.) |                                       |
| 100                                            | 0                                 | 0                                              |                      |                    | 10+                                   |
| 100                                            | 10                                | 10.0                                           | 250                  | 8                  | 4                                     |
| 100                                            | 10                                | 10.0                                           | 175                  | 8                  | 3+                                    |

<sup>1</sup> Stabilization reaction carried out with a blend of 10 weight percent of product A in the base stock.

<sup>2</sup> The lead acetate test in this example was carried out as described in Example I.

It will be noted that the evolution of H<sub>2</sub>S from the compositions containing product A was substantially reduced by treating the compositions with PbO<sub>2</sub> in accordance with the present invention.

When the stabilized products, particularly the stabilized phosphosulfurized hydrocarbons, of the present invention are employed in lubricating oils, they are generally added in proportions of about 0.1 to about 10.0% and preferably about 1.0 to about 6.0%, based on the total composition. The proportions giving the best results will vary somewhat according to the nature of the additive and the specific purpose which the lubricant is to serve in a given case. For commercial purposes, it is convenient to prepare concentrated oil solutions in which the amount of the stabilized additive in the composition ranges from 25% to 75% by weight, and to transport and store them in such form. In preparing a lubricating oil composition for use as a crankcase lubricant, the additive concentrate is merely blended with the base oil in the required amount.

The products of the present invention may be employed not only in ordinary hydrocarbon lubricating oils but also in the "heavy duty" type of lubricating oils which have been compounded with such detergent type additives as metal soaps, metal petroleum sulfonates, metal phenates, metal alcoholates, metal alkyl phenol sulfides, metal organo phosphates, phosphites, thiophosphates, and thiophosphites, metal xanthates and thioxanthates, metal thiocarbamates, and the like. Other types of additives, such as phenols and phenol sulfides, may also be present.

The lubricating oil base stock used in the compositions of this invention may be straight mineral lubricating oils or distillates derived from paraffinic, naphthenic, asphaltic or mixed base crudes, or, if desired, various blended oils may be employed as well as residuals, particularly those from which asphaltic constituents have been carefully removed. The oils may be refined by conventional methods using acid, alkali and/or clay or other agents such as aluminum chloride, or they may be extracted oils produced by solvent extraction with solvents such as phenol, sulfur dioxide, etc. Hydrogenated oils or white oils may be employed as well as synthetic oils prepared, for example, by the polymerization of olefins or by the reaction of oxides of carbon with hydrogen or by the hydrogenation of coal or its products. In certain instances cracking coal tar fractions and coal tar or shale oil distillates may also be used.

Synthetic lubricating oils having a viscosity of at least 30 S. S. U. at 100° F. may also be used, such as esters of monobasic acids (e. g. the ester of C<sub>8</sub> Oxo alcohol with C<sub>8</sub> Oxo acid; the ester of C<sub>13</sub> Oxo alcohol with octanoic acid, etc.), esters of dibasic acids (e. g. di-2-ethyl hexyl sebacate, di-nonyl adipate, etc.), esters of glycols (e. g. C<sub>13</sub> Oxo acid diester of tetraethylene glycol, etc.), complex esters (e. g. the complex ester formed by reacting one mole of sebacic acid with two moles of tetraethylene glycol and two moles of 2-ethyl-hexanoic acid; the com-

plex ester formed by reacting one mole of tetraethylene glycol with two moles of sebacic acid and two moles of 2-ethyl hexanol; the complex ester formed by reacting together one mole of azelaic acid, one mole of tetraethylene glycol, one mole of C<sub>8</sub> Oxo alcohol, and one mole of C<sub>8</sub> Oxo acid), esters of phosphoric acid (e. g. the ester formed by contacting three moles of the mono methyl ether of ethylene glycol with one mole of phosphorus oxychloride, etc.), halocarbon oils (e. g. the polymer of chlorotrifluoroethylene containing twelve recurring units of chlorotrifluoroethylene), alkyl silicates (e. g. methyl polysiloxanes, ethyl polysiloxanes, methyl-phenyl polysiloxanes, ethyl-phenyl polysiloxanes, etc.), sulfite esters (e. g. ester formed by reacting one mole of sulfur oxychloride with

10 two moles of the methyl ether or ethylene glycol, etc.), carbonates (e. g. the carbonate formed by reacting C<sub>8</sub> Oxo alcohol with ethyl carbonate to form a half ester and reacting this half ester with tetraethylene glycol), mercaptals (e. g. the mercaptal formed by reacting 2-ethyl hexyl mercaptan with formaldehyde), formals (e. g. the formal formed by reacting C<sub>13</sub> Oxo alcohol with formaldehyde), polyglycol type synthetic oils (e. g. the compound formed by condensing butyl alcohol with fourteen units of propylene oxide, etc.), or mixtures of any of the 15 above in any proportions. Also, mixtures of these synthetic oils and mineral oils in any proportions may be employed. Also, for special applications, animal, vegetable or fish oils or their hydrogenated or voltalized products may be employed in admixture with the synthetic 20 and/or mineral oils.

For the best results the base stock chosen should normally be an oil which with the new additive present gives the optimum performance in the service contemplated. However, since one advantage of the additives 25 is that their use also makes feasible the employment of less satisfactory mineral oils, no strict rule can be laid down for the choice of the base stock. The additives are normally sufficiently soluble in the base stock, but in some cases auxiliary solvent agents may be used. The 30 lubricating oils will usually range from about 40 to 150 seconds (Saybolt) viscosity at 210° F. The viscosity index may range from 0 to 100 or even higher.

Other agents than those which have been mentioned 35 may be present in the oil composition, such as dyes, pour point depressants, heat thickened fatty oils, sulfurized fatty oils, sludge dispersers, antioxidants, thickeners, viscosity index improvers, oiliness agents, resins, rubber, olefin polymers, and the like. Assisting agents which are particularly desirable as plasticizers and defoamers 40 are the higher alcohols having preferably 8 to 20 carbon atoms, e. g. octyl alcohol, lauryl alcohol, stearyl alcohol, and the like.

In addition to being employed in lubricants, the additives of the present invention may also be used in other 45 mineral oil products such as motor fuels, hydraulic fluids, torque converter fluids, cutting oils, flushing oils, turbine oils, transformer oils, industrial oils, process oils, and the like, and generally as useful additives in oleaginous products. They may also be used in gear lubricants, 50 greases and other products containing lubricating oils as ingredients.

What is claimed is:

1. An odor stabilized organic product obtained by treating a phosphorus sulfide treated olefin polymer with PbO<sub>2</sub> at an elevated temperature in the range of 80° to 400° F. for a time in the range of 8 to 24 hours.
2. A stabilized organic product obtained by treating a phosphorus sulfide treated olefin polymer with about 5 to 30% by weight of PbO<sub>2</sub> at a temperature of about 55 150° to 350° F. for about 8 to 24 hours.
3. A stabilized organic product obtained by treating a P<sub>2</sub>S<sub>5</sub> treated polyisobutylene having a molecular weight of about 500 to 2,000 with about 10 to 20% by weight of PbO<sub>2</sub> at about 300° F. for about 12 to 16 hours.
4. A method for reducing the evolution of hydrogen 60

sulfide from a phosphorus sulfide treated olefin polymer which comprises treating said phosphorus sulfide treated polymer with about 5 to 30% by weight of finely divided  $PbO_2$  at a temperature of about  $150^{\circ}$  to  $350^{\circ}$  F. for about 8 to 24 hours.

5. A method for reducing the evolution of hydrogen sulfide from a  $P_2S_5$  treated polyisobutylene having a molecular weight of about 500 to 2,000 which comprises treating said  $P_2S_5$  treated polyisobutylene with about 10 to 20% by weight of finely divided  $PbO_2$  at about  $300^{\circ}$  F. for about 12 to 16 hours, and removing unreacted  $PbO_2$  from the resultant reaction mixture.

## References Cited in the file of this patent

## UNITED STATES PATENTS

|              |                      |               |
|--------------|----------------------|---------------|
| 1,963,084    | Gardner et al. ----- | Dec. 2, 1931  |
| 5 2,315,529  | Kelso -----          | Apr. 6, 1943  |
| 2,356,074    | May -----            | Aug. 15, 1944 |
| 2,381,907    | Hughes -----         | Aug. 14, 1945 |
| 2,424,402    | Loane -----          | July 22, 1947 |
| 10 2,460,041 | Sparks -----         | Jan. 25, 1949 |
| 2,606,182    | Musselman -----      | Aug. 5, 1952  |
| 2,643,248    | Brennan -----        | June 23, 1953 |
| 2,773,860    | Musselman -----      | Dec. 11, 1956 |